# EUROPEAN PATENT SPECIFICATION

(11) **EP 0 050 397 B1**
(45) Date of publication and mention of the grant of the patent: **05.09.1984**
(21) Application number: 81302057.5
(22) Date of filing: 08.05.1981
(51) Int. Cl.: B22D 11/01, B22D 11/06, C22C 38/00, H01F 1/14

(54) **Cast metallic strip and method and apparatus for producing same**
Gegossenes metallisches Band sowie Verfahren und Einrichtung zu dessen Herstellung
Billette métallique coulée et procédé et appareil pour sa fabrication

(30) Priority: 22.10.1980 US 199149
(43) Date of publication of application: 28.04.1982
(73) Proprietor: WILKINSON SWORD LIMITED, High Wycombe Buckinghamshire HP13 6EJ (GB)
(72) Inventor: Ward, Brian Laurance, Knapp Hill Woking Surrey (GB)
(74) Representative: Sheader, Brian N.

## Description

The present invention relates to a rapidly quenched cast metallic strip and to a method and apparatus for producing such strip.

This invention is directed to metallic strip materials, whether amorphous, crystalline or combinations thereof, having dissimilar portions. In a preferred embodiment this invention relates to metal alloys in strip form, at least a portion of which are amorphous. In this specification the term "amorphous" is intended to refer to a composition in which at least 50% is amorphous, which is typically measured by X-ray defraction.

Since the early 1900's it has been taught, such as in United States Patents Nos. 905,758 and 993,904, that metallic strip material could be continuously produced by delivering molten metal to. a moving chill surface. More recent developments, such as United States Patent No. 4,142,571, teach specific refinements in strip casting nozzle structure to aid in the production of strip material. Also, various references, including United States Patent No. 3,856,513, disclose preferable alloys, particularly for the production of amorphous strip and wire material.

For certain applications, it has been found beneficial to join at least two sheets of strip material along their longitudinal edges. Such joining can be used to obtain a strip having a greater overall width, or can be used to join dissimilar portions, e.g., portions of dissimilar composition. Common techniques for joining a plurality of strips include welding, brazing and soldering. However, certain factors, including the heat, and particularly the heat gradient, generated in welding, brazing and soldering can adversely affect the quality of the composition of one or more said portions or the quality of the mutliplex strip material so produced.

As mentioned above, a preferred embodiment of the present invention pertains to strip material in which at least one dissimilar portion is amorphous. Amorphous metal alloys are those produced by a process in which crystallization is avoided, typically by extremely rapidly quenching the metal from the liquid state. Such cooling rate is usually of the order of at least 104°C per second. Because of their atomic arrangement and composition, some amorphous alloys can possess enhanced properties, including higher strength and increased resistance to chemical attack when compared to conventional crystalline alloys. Therefore, such amorphous alloys may be ideally suited for uses including but not limited to razor blade edge materials due to their properties of strength, hardness, ductility and corrosion resistance. Certain amorphous materials are also known to possess enhanced magnetic and electrical properties and the strip of the present invention may be desirable for electrical end uses.

The present invention applies equally to rapidly cast crystalline metallic materials which have a multitude of uses. The present invention further comprehends combinations of dissimilar crystalline metallic materials, dissimilar amorphous metallic materials and combinations thereof where it is desirable to utilize such dissimilar materials to decrease the overall cost of the composite, or multiplex strip, or to localize desired properties, gauge, etc. of dissimilar materials in a composite strip. For example, the present invention may be utilized to produce delicate material by simultaneously providing edge portions of a more rugged material which would facilitate the handling of the delicate material. After production, the handling portions could easily be trimmed from the strip. Also, this invention could be utilized to join alloys which exhibit different thermal electric properties, suitable for use in the production of thermocouples or multiple thermocouples. Additionally, the present invention may be employed to cast strip having varying gauges across the width thereof to intentionally vary the mechanical strength, electrical properties, etc. across the width of the strip. Further, this invention can be used to produce strip having alloys of various expansion characteristics across the width thereof. Thus, by heating such strip an intentional curvilinear strip configuration may be obtained. It should be understood that a variety of applications can be made of the strip of this invention, and that the above examples are merely illustrative and should not be interpreted as limiting the scope of this invention in any manner.

Accordingly, a new and improved multiplex strip material is desired in which dissimilar portions are joined in a fashion which does not adversely affect either the overall quality of such individual strip components or the integrity of each of such strips. Likewise, a new and improved method and apparatus for producing such strip components and multiplex combinations is desired.

German Offenlegungsschrift No., 2,856,795 discloses a number of embodiments of metallic strip manufacture by delivering to a rotating chill drum from multi-orifice nozzles a plurality of melt streams which run or fuse together. It discloses that a double-layer strip of two dissimilar metals can be made by depositing a first metal stream on to the chill drum and thereafter depositing a second metal stream to form a second layer over, and co-extensive with, the cast first stream.

The present invention provides a rapidly quenched, cast metallic strip comprising a plurality of dissimilar rapidly quenched, cast metallic portions, each portion metallurgically alloy-bonded during casting to an adjacent portion along the longitudinal extent of said strip, wherein said plurality of portions are dissimilar portions of at least two different compositions, and each portion is metallurgically alloy-bonded during casting to a laterally adjacent dissimilar portion along the adjacent edges of said dissimilar portions.

The present invention also provides a method of casting metallic strip having a plurality of dissimilar portions metallurgically alloy-bonded along the longitudinal extent of said strip, comprising delivering a plurality of streams of molten metal from a plurality of nozzles onto a rapid quenching casting surface moving at a rate of from 61 to 3048 metres (200 to 10,000 linear surface feet) per minute past said nozzles characterised by depositing a first stream of a first molten metal onto said casting surface from a nozzle of a first crucible and depositing laterally of the first at least one additional stream of a second, different molten metal from a nozzle of a second crucible onto said casting surface such that a peripheral edge portion of said at least one additional stream contacts a peripheral edge portion of adjacent different metal to create a metallurgical alloy-bond therebetween during casting.

The present invention further provides apparatus for casting metallic strip having a plurality of dissimilar portions metallurgically alloy-bonded along the longitudinal extent of said strip, comprising crucible means for receiving and holding molten metal and having a plurality of nozzles through which a plurality of streams of molten metal can be delivered from said means to a rapid quenching casting surface located within 3.048 mm (0.120 inch) of the nozzles and movable past the nozzles at a speed of from 61 to 3048 metres (200 to 10,000 linear surface feet) per minute, wherein said crucible means comprises a first crucible having an internal cavity for receiving and holding molten metal and a nozzle through which a first stream of molten metal can be delivered from its cavity and deposited onto the casting surface, and at least one additional crucible having an internal cavity for receiving and holding molten metal and a nozzle through which at least one additional stream of a second, different molten metal can be delivered from its cavity and deposited onto the casting surface, said at least one additional crucible having the nozzle thereof disposed laterally of the first such that a peripheral edge portion of said at least one additional stream will contact a peripheral edge portion of adjacent different metal to create a metallurgical alloy-bond therebetween during casting.

Among the advantages of the present invention is the ability to combine a plurality of dissimilar portions into a composite strip material with a metallurgical alloy-bond between adjacent dissimilar portions which is created during the casting of such strip material without adversely affecting the quality or properties of the individual strip portions.

Another advantage of the present invention is that it enables a strip of rapidly cast material to be provided having at least two 'dissimilar portions metallurgically alloy-bonded along the length of the strip thereby forming a multiplex strip,. or composite strip, exhibiting different properties, structure or quality in each portion of the strip.

Another advantage of the present invention is the provision of a method and an apparatus for rapidly casting a strip comprised of dissimilar portions metallurgically alloy-bonded to one another along the length of the strip during casting operations without adversely affecting the quality or the properties of the strip material.

It follows that a further advantage of the present invention is that where strength, corrosion resistance and other qualities are required only at an edge or at the edges of the strip material, the expensive alloying ingredients, such as cobalt and molybdenum only have to be used at such edge portions of a multiplex strip material, thus reducing the cost of the strip.

Another advantage of this invention is that it enables a strip of metallurgically alloy-bonded amorphous and crystalline metallic portions to be provided without causing the amorphous portion to crystallize during the bonding thereof The invention also enables a metallic strip to be provided of components joined at a transition zone wherein an alloy formed at the transition zone has enhanced properties over those of the joined portions.

This invention will be more fully understood and appreciated with reference to the accompanying drawings, in which:-
Figure 1 is a front cross-sectional view of an apparatus of the present invention.
Figure 2 is an enlarged cross-sectional view of the nozzle area of the apparatus shown in Figure 1.
Figure 3 is a partial perspective view illustrating an alternative apparatus of the present invention.
Figure 4 is a perspective view of the casting surface and the strip cast thereon from the apparatus shown in Figure 3.
Figure 5 is a top elevation view of an alternative apparatus of the present invention.
Figure 6 is a perspective view of an alternative apparatus of the present invention.
Figure 7 is a cross-sectional view of a preferred crucible and nozzle for use in apparatus of the present invention.
Figure 8 is a graph of an energy dispersion X-ray analysis for the element nickel taken across the strip of the Example which appears hereinafter.
Figure 9 is a graph of an energy dispersion X-ray analysis for the element silicon taken across the strip of the said Example.
Figure 10 is a graph of the Knoop hardness at a load of 200 grams taken across the strip of the said Example.

Referring particularly to the drawings, Figures 1 and 2 illustrate a preferred apparatus of the present invention. As shown in Figure 1 this apparatus includes a first crucible 10 and a second crucible 11 each having an internal cavity designed to receive and hold metal. The first crucible 10 also includes an orifice or nozzle 10a through which a first stream of molten metal can be delivered from the cavity of the crucible 10 to a casting surface 18 whilst the second crucible 11 likewise includes an orifice or nozzle 11 a through which a second stream of molten metal can be delivered from the cavity of the crucible 11 to the casting surface 18. In a preferred embodiment the continuous strip material 30 (Figs 3, 4 and 6) is cast on a relatively smooth outer peripheral surface 18 of a circular drum or wheel 13. It should be appreciated that configurations other than circular may be employed, for example, the strip of the present invention could be cast onto a moving belt as shown in Figure 6, onto the interior surface of the drum, between a pair of facing rollers, into a quench fluid, or the like.

In a preferred embodiment, the casting element 13 comprises a water cooled, precipitation hardened copper alloy wheel containing about 90% copper. Copper and copper alloys are chosen for their high thermal conductivity and wear resistance. However, steel brass, aluminum, aluminum alloys or other materials may be utilized alone or in combination or multipiece wheels having sleeves of molybdenum or other material may also be employed. Likewise, cooling may be accomplished with the use of a medium other than water. Water is chosen for the preferred embodiment for its low cost and its ready availability.

In the operation of the strip casting apparatus of the present invention, the outer peripheral surface 18 of the casting wheel 13 must be able to absorb the heat generated by contact with molten metal at the initial casting point, and such heat must diffuse substantially into the copper wheel during each rotation of the wheel. Removal of the diffused heat may be accomplished, for example, by delivering a sufficient quantity of water through internal passageways located near the periphery of the casting wheel 13. Alternatively, the cooling medium may be delivered to the underside of the casting surface. Understandably, refrigeration techniques and the like may be employed to adjust and optimize cooling rates, for example, to effect wheel expansion or contraction during strip casting.

Whether a drum, wheel or belt is employed for casting, the casting surface 18 should generally be smooth and symmetrical to maximize uniformity in strip casting. For example, in certain strip casting operations wherein it is desired to cast uniform gauge strip, the distance between the outer peripheral casting surface 18 and the surfaces defining the orifice of the nozzle 10a or 1 a which is feeding the molten material onto the casting surface 18 should not substantially deviate from a desired or set distance. This distance shall hereinafter be called the standoff distance or gap. It is understandable that the gap at each nozzle should normally be substantially maintained constant throughout the casting operation when it is the intention of the operator to cast uniform gauge strip portions from that nozzle. If, however, controlled variations of thickness are desired either in the complete composite or in certain component strips of the composite, then a programmed standoff distance both for the whole nozzle component array and/or for each contributing nozzle may be employed.

It should also be understood that if the casting element is a drum or a wheel, the element should be carefully constructed so as not to be out-of-round during operation to ensure uniformity in strip casting. Along these lines, it has been found that a drum or wheel which is out-of-round by about 0.508 mm (0.020 inch), or more may have a magnitude of dimensional instability which, unless corrected or compensated during operation, may be unacceptable for certain strip casting operations. It has also been found that acceptable dimensional symmetry may be accomplished by fabricating a wheel or drum from a single, integral slab of cold rolled or forged copper. However, as mentioned above alternative materials may be employed.

The molten materials to be cast in the apparatus described herein are preferably retained in crucibles or tundishes each of which is provided with a corresponding nozzle. The nozzle is typically, though not necessarily, located at a lower portion of the crucible as shown in the drawings. The nozzle may be an integral part of the crucible, or may constitute a separate material affixed into the crucible.

Each crucible is constructed for receiving and holding molten metal therein. It will be appre-. ciated that appropriate materials must be utilized for the crucible to withstand the molten metal conditions, and where the crucible is not a monolithic structure, the joints and seams between separate pieces of the crucible must be assembled to prevent molten metal leakage during sustained operation.

One preferred crucible 10 for continuous production of rapidly cast strip material is illustrated in detail in Figure 7. It should be understood that the molten metal holding portion of the crucible 10, which is formed between the inside surfaces, may take a variety of forms or shapes. However, in a preferred embodiment an upper portion of the crucible 10 has a significantly larger cross-sectional volume than that of the nozzle area of the crucible 10 in order that the molten metal head height, above the nozzle 10a, is substantially unaffected by minor variations in molten metal in the crucible 10. Such structure contributes to the maintenance of a substantially constant metallostatic head pressure at the nozzle, even with minor variations in metal volume that may occur in the crucible 10 in sustained or continuous casting operations. It should be appreciated that casting may also be effected under externally applied pressure using equipment which could be directly controlled.

As shown in Figure 7, it is also preferable that the inside surfaces of the crucible 10 converge toward one'another in the direction of the nozzle 10a, and that such inside surfaces be radiused, rounded or generally curvilinear at locations of turns or bends in the crucible 10 to minimize metal turbulence therein during a casting operation.

The molten metal holding area, formed between the inside surfaces of the crucible 10 shown in Figure 7 should be enclosed, such as with sidewalls. It is noted that the width of the crucible nozzles of the present invention should not be limited. It has been found that a crucible 10 and nozzle 1 Oa of the present invention may be constructed by first cutting or carving refractory boards, such as insulating boards made from fiberized kaolin, into the desired shape, such as that shown in Figure 7. Any number of these boards may be stacked upon one another to obtain the desired crucible 10 and nozzle 10a width. There is not expected to be a restriction on the maximum width of the crucible and nozzle of the present invention, and widths in excess of 914 mm (thirty six inches) for strip portions from one crucible are comprehended by the present invention. After the requisite number of boards are stacked, the inside surfaces may be sanded or otherwise finished to provide generally smooth inside surfaces across the width of the stacked elements forming the crucible 10. It should also be understood that single piece materials may be used to construct a monolithic crucible in which case stacking would not be necessary. After the carved boards are stacked, the stack may be disposed between uncarved boards, which may serve as the sidewalls for the crucible 10.

To hold the stacked boards, including the sidewalls in position, it has been found convenient to dispose a metal plate against the outside surface of each sidewall and to bolt the plates together at a suitable number of locations about the crucible, thereby tightly compacting the crucible assembly. With such assembly, a minor amount of molten metal may tend to flow into the seams between the boards, but the compaction of the assembly causes the metal to freeze, and thereby arrests the flow before it adversely affects the crucible or the strip casting operation. It should be understood that the crucible may be assembled with refractory cements, or the like, or may be constructed of a monolithic structure which does not require assembly.

As discussed above, a nozzle is located in each crucible, preferably in a lower portion thereof. The nozzle comprises an orifice passage defined between inside surfaces of the crucible. In a preferred embodiment as illustrated in Figure 7, the nozzle 10a is formed between a crucible surface and an inside surface of an insert 50. A portion of the inside surface of the insert 50, is preferably disposed against a portion of a ridge formed by an outside surface of the crucible 10.

It should be appreciated that the insert 50, described in a preferred crucible, may be easily replaced, although it is preferred that the insert 50 and the crucible be reused, either together or separately. It should also be noted that damage to an insert 50 shall not render the entire crucible unserviceable. In the event of such insert damage, the insert 50 is merely replaced and the process may continue.

In a preferred embodiment, as shown in cross-section in Figure 7, the insert 50 is provided with a front edge surface 70. In such embodiment, the front edge surface 70 faces the casting surface 18 and is disposed to within less than 3.048 mm (0.120 inch) of the casting surface 18. Preferably, the front edge surface 70 is disposed to within 2.032 mm (0.080 inch) and in a more preferred embodiment, to within 0.508 'mm (0.020 inch) of the casting surface 18. It is also preferred that in such embodiment the front edge surface 70 be in substantially complete parallelism with the casting surface 18. Such complete parallelism may be accomplished by placing a sheet of sandpaper, or the like, against the casting surface 18 with the grit side of the sandpaper facing the insert 50. By moving the insert 50 into tight contact with the casting surface 18, with the sandpaper disposed therebetween, and by moving the casting surface and sandpaper simultaneously past the insert 50, the front edge surface 70 is ground by the grit side of the sandpaper into substantially complete parallelism with the casting surface 18. Such substantially complete parallelism may be achieved even when round or other curvilinear casting surfaces are employed. To achieve such parallelism by this procedure 400 to 600 grit sandpaper has been found to be adequate. Other surfaces of the crucible may be brought into substantially complete parallelism with the casting surfaces 18 by this same procedure.

By maintaining the front edge surface 70 in substantially complete parallelism with the casting surface 18, the standoff distance, or gap, between the front edge surface 70 and the casting surface 18 is maintained throughout the length thereof. It has been found that the gap between the front edge surface 70 and the casting surface 18 should be maintained at less than 3.048 mm (0.120 inch) in order to successfully cast strip material. Preferably, this gap is maintained at less than 2.032 mm (0.080 inch) and for casting certain alloys into thin gauge strip, gaps less than 0.508 mm (0.020 inch) are preferred. Alternatively, the corner of the insert 50 may come to a point at the front edge 70 at a 90° junction of the front edge of the insert 50, as opposed to a defined surface length as discussed above.

What is preferred with respect to the bottom surface of the nozzle 10a is that such surface be disposed as close as possible to the casting surface 18, without causing any interference for the movable casting surface therebelow. Accordingly, such surface of the nozzle may just clear the casting surface 18, i.e., be perhaps within about 0.0508 mm (.002 inch) thereof. Such spacing must not be large enough to allow significant molten metal backflow between the bottom surface of the nozzle 10 and the casting surface 18 during casting. It should be understood that provision may have to be made for edge portions of strip material which may have to pass under a portion of another downstream crucible.

Whilst the above description has been of the crucible 10 and nozzle 10a it will be understood that this description is equally applicable to the crucible 11 and nozzle 11 a.

The crucibles 10 and/or 11 are preferably constructed of a material having superior insulation ability. If the insulating ability is not sufficient to retain the molten material at a relatively constant temperature, auxiliary heaters such as induction coils 12 may have to be provided in and/or around the crucibles 10 and/or 11, or resistance elements such as wires may be provided. A convenient material for the crucibles is an insulating board made from fiberized kaolin, a naturally occurring, high purity, alumina-silica fire clay. Such insulating material is available under the trade mark Kaowool HS board. However, for sustained operations, and for casting higher melting temperature alloys, various other materials may have to be employed for constructing the crucible or the nozzle of the crucible including silica, alumina, graphite, alumina graphite, clay graphite, fire clay, quartz, boron nitride, silicon nitride, boron carbide, silicon carbide, zirconia, stabilized zirconia silicate, magnesia, chrome magnesite and various combinations or mixtures of such materials.

Although other materials are comprehended by the present invention, the insert 50 forming part of the nozzle of the crucible is preferably constructed of boron nitride, silicon nitride, silicon carbide, boron carbide, zirconia or quartz.

It is imperative that the orifice passage of the nozzle 1 Oa or 11 a remain open and its configuration remain substantially stable throughout a strip casting operation. It is understandable that the nozzles should not erode or clog, significantly, during a multiplex strip casting sequence or certain objectives such as maintaining uniformity in the casting operation and of minimizing metal flow turbulence in the crucibles may be defeated. Along these lines, it appears that certain insulating materials may not be able to maintain their dimensional stability over long casting periods. To obviate this problem the nozzle 10a or 11 a, especially that portion defined by an insert 50, may be constructed of a material which is better able to maintain dimensional stability and integrity during exposure to high molten metal temperatures for prolonged time periods. Hence the preference for the materials mentioned above.

The drive system and housing for the drum, wheel or other casting surface 16 of the present invention should be rigidly constructed to permit drum rotation without structural instability which would cause the drum to slip or vibrate. In particular, care should be taken to avoid resonant frequencies at the operating speeds for the drum. The casting surface 18 should be capable of moving at a surface speed of from 61 metres (200 linear surface feet) per minute to more than 3048 metres (10,000 linear surface feet) per minute. When utilizing a drum having a circumference of about 2.4 metres (8 feet), this rate calculates to a drum speed from about 25 rpm to about 1250 rpm. A three horsepower variable speed reversible, dynamically braked motor provides an adequate drive system for an integral copper casting drum 50 to 254 mm (2 to 10 inches) thick and about 2.4 metres (8 feet) in circumference. Power requirements may have to be modified depending upon the type and size of casting surface 18 employed. It should be appreciated that the casting surface 18 can be moved in a direction opposite to that illustrated in the drawing, and that the crucible may be disposed at any location about a circular casting wheel.

In one embodiment, the casting surface 18 on the wheel or drum of the apparatus of the present invention is smooth. It has been found that in certain applications, such as for producing amorphous strip portions, finishing the peripheral surface 18 of a casting wheel 13 with 400-grit sandpaper and preferably with 600-grit sandpaper may yield improved product uniformity.

In an exemplary operation of the apparatus of the present invention, such as illustrated in Figures 1 or 3, molten metal is delivered to a first, heated crucible 10 and into a second crucible 11, although such metal delivery may be sequential rather than simultaneous. It is understood that a heater, such as induction coils or resistance wire 12, may be provided in and/or about the crucibles 10 and 11 to obtain or to maintain relatively constant molten metal temperatures as may be desired. In the operation of the apparatus of this invention metal may be poured directly into preheated crucibles. Such metal preheat temperature and the heating of the crucibles by auxiliary devices should prevent freezing or clogging of the nozzle during the initial casting operation, and the temperature of the flowing metal should thereafter keep each crucible at sufficient temperature to ensure uninterrupted molten metal flow through each nozzle. In certain applications, the nozzle should be externally heated throughout the casting operation. Also, the metal which is fed to the crucibles may be superheated to allow a certain degree of temperature loss without adversely affecting metal flow.

In one embodiment a metallostatic head height in the crucibles should be maintained at a relatively constant level throughout the casting operation to ensure that a relatively constant static head pressure is maintained at the nozzles. This may be accomplished by initially pouring the molten metal into each crucible to the desired height and thereafter controlling the rate at which additional molten metal is poured into that crucible to maintain the metallostatic head. It is understandable that the rate at which additional molten metal is fed to the crucible should be in substantial conformity with the rate at which metal flows from the nozzle onto the casting surface 18 in forming the multiplex strip material of the present invention. Maintenance of a relatively constant height of metal in the crucibles assures that the molten metal flow pressure through the respective nozzle is maintained relatively constant so as not to adversely affect the casting operation or the quality of the strip material. Alternatively, as mentioned above, externally applied pressure may be employed to control the pressure at the nozzles.

In the present invention, a rapidly quenched metallic strip 30 is cast onto a casting surface 18. Such strip material 30 comprises a plurality of dissimilar portions, such as portions a, b, c and d in Figure 5 or portions a" b, and a₂ in Figure 6. Each individual portion of the strip 30 is metallurgically alloy-bonded to the edges of adjacent portions along the longitudinal extent of the strip. Further, such metallurgical alloy-bonding occurs as an integral part of the strip casting operation.

Strip 30 having a plurality of dissimilar portions is called "multiplex strip" or "composite strip" in this application. The multiplex strip 30 of the present invention is intended to comprehend a strip having at least two dissimilar metallic materials metallurgically alloy-bonded together along the longitudinal extent of the strip. This metallurgical alloy-bdnd occurs during the casting operation which forms the strip. The "at least two different materials" refers to different metallic compositions. However, such expression should also comprehend a multiplex strip which additionally has other properties which are different, including, but not limited to, electrical resistivity, permeability, conductivity, core loss characteristics, yield strength, hardness, atomic arrangement, gauge, corrosion resistance, thermal expansion, colour and the like.

For purposes of illustration, one portion of a multiplex strip of the present invention may have expansion characteristics different from that of a bonded, adjacent portion. Thus, by heating or cooling such strip, an intentional curvilinear strip material may >be obtained. Also, the present invention may be employed to produce multiplex strip having amorphous strip portions metallurgically alloy-bonded to crystalline strip portions. When a strip of amorphous material is joined by conventional means, involving heating, such as welding, to a strip of crystalline material the amorphous strip becomes very brittle since the temperature to which it is exposed exceeds the crystallization temperature. By the present invention, however, the quench rate may be so rapid that crystallization of the amorphous strip portion is substantially avoided, except possibly at the transition zone.

The rapid quenching of a strip casting operation may also be beneficial in the production of certain crystalline strip materials. Fast quenched crystalline alloys, in general, typically develp a highly desirable microstructure which is finer than conventionally produced crystalline materials. Also, rapidly cast crystalline materials may contain desirable alloy phases not found in conventional crystalline materials, and, conversely, rapid casting may avoid or inhibit the formation of adverse alloy phases. Additionally, rapid casting can. produce new alloy phases in crystalline materials which although they are metastable, typically exhibit improved properties.

In one preferred embodiment, the present invention pertains to the manufacturing of multiplex strip 30 having an amorphous alloy portion which is formed with an adjacent metal or metal alloy portion, which may or may not be amorphous, the latter portion being integral with the first mentioned amorphous alloy portion. In the present invention the multiple strip portions may be cast simultaneously adjacent one another onto the casting surface 18, as shown in the embodiment illustrated in Figures 1 and 2. In this embodiment, the multiple nozzles 1 Oa and 11 a each deposit a stream of molten metal 20 and 22, respectively, onto approximately the same transverse line across the casting surface 18, adjacent to one another. As best shown in Figurè2 the molten streams of metal converge to join one another and an actual alloying of the two converging streams actually occurs at the interface, also called the transition zone. It will be appreciated that the quench rate is so rapid in the casting of metallic strip material, that the merging streams do not experience sufficient residence time to significantly adversely affect the integrity of either metallic stream outside of the transition zone. Therefore, the composition gauge, hardness, strength, ductility, corrosion resistance and other properties of one portion of the strip are not adversely affected by the contact between adjacent portions even in their molten state.

Alternatively, the multiple strip portions may be cast successively onto the casting surface 18 as shown in the embodiments illustrated in Figures 3 and 4. In such embodiment, a stream of molten metal is fed from one crucible 10 onto the casting surface 18. A second crucible 11 is located downstream of the first crucible 10 with respect to the casting direction illustrated by the arrow in Figure 3. The second crucible 11 has a nozzle 11 a which must be disposed such that a peripheral edge portion of the second stream of metal contacts a peripheral edge portion of the first metal to create a metallurgical alloy-bond therebetween during casting. It will be appre- . ciated that the first stram may be molten, partially solidified or even totally solidified when the second stream contacts the peripheral edge. What is required by the casting operation is that a metallurgical alloy-bond be created therebetween as the multiplex strip is formed.

Although the development has been discussed with relation to two streams of metal to produce a duplex strip, it should be understood that any number of dissimilar portions may be metallurgically alloy bonded together in the present invention. For example, Figure 5 illustrates a multiplex strip composed of four portions a, b, c and d cast from four separate crucibles A, B, C, D. Also Figure 6 illustrates a triplex strip which may be cast by disposing two streams of metal from two separate nozzles in a common crucible A adjacent both edge portions of a single strip portion, b, from tundish B to produce a multiplex strip having portions a,, b, and a₂ metallurgically alloy-bonded during casting. It will be appreciated that in this embodiment the two nozzles of crucible A are preferably separated by a bridge of approximately the same width as the central strip portion b.

In forming the metallurgical alloy-bond between adjacent dissimilar portions, such dissimilar strip portions are fused to one another. The joint between adjacent dissimilar portions, which is called the "transition zone" throughout this application, normally extends through the strip from its upper face to its lower face in a direction substantially parallel to the longitudinal axis of a strip. Although the transition zone is illustrated in chain lines in the drawings, it should be understood that such transition zone may not be readily discernable to ordinary observation.

One preferred embodiment of this invention may be directed to the production of razor blade stock. In such embodiment the composition of the metal in the first crucible 10 is preferably chosen to produce an amorphous alloy having properties of strength, hardness, ductility and corrosion resistance, which properties are generally desirable for forming a razor blade cutting edge portion. The composition of the metal in the second crucible 11 may be chosen to provide a suitable backing material for the cutting edge portion of the strip.

### Example

A two-piece, or duplex, metal alloy strip was formed in accordance with the present invention using two crucibles, similar to that illustrated in Figure 3. The casting surface comprised a 3.8 cm peripheral surface of a 20 cm diameter copper wheel rotated at a speed of 32 metres per second with the axis of rotation being substantially horizontal. In this example the crucible located slightly downstream with respect to the other crucible shall be referred to as the "first crucible". The first crucible 11 was made of silica and had a generally circular cross-section with an internal diameter of 10 mm tapering to a slit nozzle with internal dimensions of 5 mm by 0.42 mm. The bottom surface of the nozzle was maintained at about 0.43 mm above the casting surface, and the nozzle was disposed substantially parallel to the axis of the wheel. The first crucible 11 contained about 8.4 grams of an alloy composition Fe₈₃ Si₅ B,₂, based on an atomic percent. This alloy is hereinafter called Alloy 1.

The second crucible 10, also made of silica, was of circular cross-section with an internal diameter of 10 mm, tapering through 24 mm to a circular orifice having an internal diameter of about 0.64 mm. The bottom surface of the nozzle was maintained at about 0.43 mm above the casting surfce. The second crucible 10 was displaced about 5 mm from the first crucible in a direction opposite to the rotation of the wheel. The second crucible 10, contained about 5.6 grams of an alloy composition Feo Ni₄ₒ B₂₀, based on atomic percent. The alloy is hereinafter called Alloy II.

One edge of the nozzle orifice of the second crucible 10 was disposed on the same circumferential line with respect to the wheel as one edge of the nozzle orifice of the first crucible, so that the two nozzle orifices would not, if transposed, substantially overlap.

In this example, both crucibles 10 and 11 lay in the general plane described by the wheel. As measured in a direction opposite to that of the rotation of the wheel, the first crucible 11 being 1.5° from the vertical and the second crucible 10 being 40° from the vertical. In this example, the crucibles were heated to about 1350°C with an induction heating coil so as to melt their contents. The atmosphere in the crucibles was argon at atmospheric pressure, although protective atmospheres are not essential in this invention. The casting surface was moved past the nozzles at a peripheral speed of 32 linear metres per second and the crucibles were simultaneously over-pressured with argon to expel their contents, the first crucible 11 at 140.6 g/cm^{z} (2 psi) and the second crucible 10 at 492 g/cm² (7 psi). A continuous duplex strip was formed which was ejected from the casting surface in about one half of one second.

The strip was flat, having a width of about 4.5 mm. The strip portion originating from the first crucible 11 was about 2.7 mm wide and about 30 µm thick with the remaining portion approximately 50 µm thick. The ribbon was ductile and when caused to fail under test, showed no preferential parting at the joint, or transition zone. Both portions of the strip in this example were amorphous.

It has been found that beyond a very small distance from the joint between the two parts of the ribbon, of the order of less than 0.5 mm, the composition of one portion is not contaminated by metals from the other. Thus, analysing for nickel on the wheel face of the strip, a bold nickel peak was observed for 1.6 mm dropping to zero peak height over a distance of 0.05 mm at the junction. See the nickel trace illustrated in Figure 8 wherein the height of the nickel trace is directly proportional to the amount of nickel in the Alloy II portion of the strip. Also, a scan for silicon had a sharp cutoff at the junction thereafter dropping to zero peak height. See the silicon trace illustrated in Figure 9 wherein the height of the silicon trace is directly proportional to the amount of silicon in the Alloy I portion of the strip. The horizontal axis of the graphs of Figures 8 and 9 connotes distance, with the traced portion extending over a full distance of approximately four millimetres.

The graph illustrated in Figure 10 shows the Knoop hardness of this strip at a load of 200 grams. This graph illustrates that the transition zone, i.e. the extent of the joint where Alloy I and Alloy II strip portions are metallurgically alloy-bonded together, has a width of about 1.15 mm. As shown in Figure 10, the strength of Alloy I and Alloy II respectively, remains substantially uniform outside the transition zone. It' is noted that although the strength of the strip at the transition zone usually has a value between the strengths of adjacent portions, with certain alloys, the metallurgical alloy-bond at the transition zone may exhibit a strength which is higher or lower than that of the adjacent portions, or the transition zone may consist of a separate alloy exhibiting other desirable properties including corrosive resistance, electrical resistivity, and the like. Thus, by approximately choosing the dissimilar alloys, a combination alloy can be formed within the transition zone. Likewise, appropriate alloys may be chosen which could produce crystalline strip portions and an amorphous transition zone, or vice versa.

In general, the transition zone metallurgically alloy-bonding dissimilar strip portions has an identifiable width of less than about 1.50 mm or less than about five times the average gauge of the bonded dissimilar portions. More preferably, the width of the transition zone is less than three times the average gauge or thickness of the bonded portions.

While particular reference has been made to a duplex strip, it is also possible to produce multiplex strips having any number of dissimilar portions, by the present invention. For example, a multiplex strip can be produced which has a composition preferred for a cutting edge of a razor blade on both margins and an intermediate broad band of material appropriate for backing the cutting edge material. Such strip may then be formed into double edge razor blades or may be split longitudinally to provide single edge blades. In another example, the cutting edge composition of stainless steel may be used for a central portion of the strip, which is subsequently split longitudinally through the central portion to provide two strips of duplex form. A possible advantage of such triplex strip is the maintenance of its form when coiled for purposes of storage and subsequent processing.

During the continuous casting of multiplex strip material, the tendency of the strip 30 to adhere to the casting surface 18 for a significant distance, such as several hundred centimetres or more, beyond the nozzle has been observed. This phenomenon is benefical in casting multiplex strip through staggered nozzles, such as shown in Figures 3, 5 and 6. However it is understandable that if the strip material remains on a rotating casting drum or wheel 13 for a full revolution, damage to the crucibles could result. It has been found that the use of a doctor blade, such as a knife type element riding at or near the drum surface 18, approximately 0.75 to 1.83 metres (2.5 to 6 feet) from the nozzle may counter such adherence. With such an arrangement, the cast strip may be removed from the drum by such doctor blade. Such doctor blade has been found particularly useful in the production of thinner amorphous strip materials which appear to have a greater tendency to adhere to the casting surface 18 than do the crystalline strip materials. It is believed that the force which retains the strip on the casting surface reflects the quality of the thermal contact between the strip and the casting surface. Alternative arrangements, such as an air knife, may also be employed to separate the strip from the casting surface.

The casting of relatively high quality multiplex strip material, possibly including amorphous strip portions, which for the purpose of this invention includes materials which are at least 50% amorphous, is feasible and practical using the apparatus and procedures described above. Understandably, the quency rates must usually be higher for amorphous material as compared to crystalline material. When necessary quench rates may be accelerated such as by increasing the speed of the casting surface, or the like.

Typical alloys which may be cast into multiplex strip in accordance with the present invention include those in which at least one portion comprises an alloy having iron, nickel, cobalt and combinations or mixtures thereof as a major constituent. Major constituents are those which dominate the composition such that no other element is present in a larger amount, based on atomic percentages. Such alloys typically contain, as minor constituents, silicon, boron, phosphorous, carbon, aluminum, vanadium, beryllium, chromium and combinations or mixtures thereof. Only incidental impurities, less than one percent, and preferably less than 0.1 %, should be present in such alloys. As mentioned above, such alloys are preferably amorphous. However crystalline alloys and combinations of crystalline and amorphous alloy portions are comprehended by the multiplex strip of the present invention. Preferred iron-base alloys for portions of the strip of this invention include the following:

## Claims

1. A rapidly quenched, cast metallic strip comprising a plurality of dissimilar rapidly quenched, cast metallic portions, each portion metallurgically alloy-bonded during casting to an adjacent portion along the longitudinal extent of said strip, characterised in that said plurality of portions (a, b, c, d; a₁, b, a₂) are dissimilar portions of at least two different compositions, and each portion is metallurgically alloy-bonded during casting to a laterally adjacent dissimilar portion along the adjacent edges of said dissimilar portions.

2. A strip according to claim 1, wherein at least two adjacent portions of said strip have a dissimilar atomic arrangement.

3. A strip according to claim 2, wherein at least one dissimilar portion of said strip is amorphous (as hereinbefore defined).

4. A strip according to claim 2 or 3, wherein at least one dissimilar portion of said strip is crystalline.

5. A strip according to any one of the preceding claims, wherein the metallurgical alloy-bond is formed at a transition zone which is amorphous (as hereinbefore defined) and wherein the dissimilar portions adjacent said transition zone are crystalline.

6. A strip according to any one of claims 1 to 4, wherein adjacent dissimilar portions are amorphous (as hereinbefore defined) and the metallurgical alloy-bond is formed at a transition zone therebetween which is crystalline.

7. A strip according to any one of the preceding claims, wherein at least one dissimilar portion of said strip is stainless steel.

8. A strip according to any one of the preceding claims, wherein at least two adjacent portions of said strip have dissimilar thicknesses.

9. A strip according to any one of the preceding claims, wherein at least two adjacent portions of said strip have dissimilar corrosion resistant properties.

10. A strip according to any one of the preceding claims, wherein at least two adjacent portions of said strip have dissimilar electrical properties.

11. A strip according to any one of the preceding claims, wherein at least two adjacent portions of said strip have dissimilar expansion characteristics.

12. A strip according to any one of the preceding claims, wherein at least one portion comprises an alloy having major constituents selected from iron, nickel, and cobalt mixtures thereof and minor constituents selected from silicon, boron, phosphorous, carbon, aluminium, vanadium, beryllium, chromium and mixtures thereof, with incidental impurities.

13. A strip according to any one of the preceding claims, wherein at least one portion is amorphous (as hereinbefore defined) and has a composition of Fe₈₀₋₈₅Si₃₋₇B₁₀₋₁₅, based on atomic percentages.

14. A strip according to any one of the preceding claims, wherein at least one portion is amorphous (as hereinbefore defined) and has a composition of Fe₃₆₋₄₃Ni₃₆₋₄₃B₁₇₋₂₂, based on atomic percentages.

15. A strip according to any one of the preceding claims, wherein at least one portion is amorphous (as hereinbefore defined) and has a composition of FesoB,2Sig, based on atomic percentages.

16. A strip according to any one of the preceding claims, wherein at least one portion is amorphous (as hereinbefore defined) and has a composition of Fe₇₉B₁₅Si₆, based on atomic percentages.

17. A strip according to any one of the preceding claims, wherein at least one portion is amorphous (as hereinbefore defined) and has a composition of Fe₈₁B₁₃Si₅C₁, based on atomic percentages.

18. A strip according to any one of the preceding claims, wherein at least one portion is amorphous (as hereinbefore defined) and has a composition of Fe₈₄B₁₅Si₁, based on atomic percentages.

19. A strip according to any one of the preceding claims, wherein the metallurgical bond is formed at a transition zone between portions having a width of less than 1.5 mm.

20. A strip according to any one of the preceding claims, wherein the metallurgical bond is formed at a transition zone between portions having a width of less than five times the average thickness of the bonded portions.

21. A strip according to any one of the preceding claims, wherein the metallurgical bond is formed at a transition zone having mechanical strength greater than that of both adjacent bonded portions.

22. A strip according to any one of the preceding claims 1 to 20, wherein the metallurgical alloy-bond is formed at a transition zone having lower mechanical strength than that of both adjacent bonded portions.

23. A method of casting metallic strip having a plurality of dissimilar portions metallurgically alloy-bonded along the longitudinal extent of said strip, comprising delivering a plurality of streams of molten metal from a plurality of nozzles onto a rapid quenching casting surface moving at a rate of from 61 to 3048 metres (200 to 10,000 linear surface feet) per minute past said nozzles, characterised by depositing a first stream (20) of a first molten metal onto said casting surface (18) from a nozzle (1 Oa) of a first crucible (10) and depositing laterally of the first at least one additional stream (22) of a second, different molten metal from a nozzle (11 a) of a second crucible (11) onto said casting surface (18) such that a peripheral edge portion of said at least one additional stream contacts a peripheral edge portion of adjacent different metal to create a metallurgical alloy-bond therebetween during casting.

24. Apparatus for casting metallic strip having a plurality of dissimilar portions metallurgically alloy-bonded along the longitudinal extent of said strip, comprising crucible means for receiving and holding molten metal and having a plurality of nozzles through which a plurality of streams of molten metal can be delivered from said means to a rapid quenching casting surface located within 3.048 mm (0.120 inch) of the nozzles and movable past the nozzles at a speed of from 61 to 3048 metres (200 to 10,000 linear surface feet) per minute characterised in that said crucible means comprises a first crucible (10) having an internal cavity for receiving and holding molten metal and a nozzle (1 Oa) through which a first stream (20) of molten metal can be delivered from its cavity and deposited onto the casting surface (18), and at least one additional crucible (11) having an internal cavity for receiving and holding molten metal and a nozzle (11a) through which at least one additional stream (22) of a second, different molten metal can be delivered from its cavity, and deposited onto the casting surface (18), said at least one additional crucible (11) having the nozzle (11 a) thereof disposed laterally of the first such that a peripheral edge portion of said at least one additional stream (22) will contact a peripheral edge portion of adjacent different metal to create a metallurgical alloy-bond therebetween during casting.

25. Apparatus according to claim 24, wherein at least one said crucible (10, 11) is constructed of a molten metal resistant material selected from silica, alumina, graphite, alumina graphite, clay graphite, fire clay, quartz, boron nitride, silicon nitride, silicon carbide, boron carbide, zirconia, stabilized zirconia silicate, magnesia, chrome magnesite, fiberized kaolin and combinations thereof.

26. Apparatus according to claim 24 or 25, wherein at least a portion of the nozzle (10a, 11a) of at least one said crucible (10, 11) is constructed of molten metal resistant material selected from silica, alumina, graphite, alumina graphite, clay graphite, fire clay, quartz, boron nitride, silicon nitride, silicon carbide, boron carbide, zirconia, stabilized zirconia silicate, magnesia, chrome magnesite, fiberized kaolin and combinations thereof.

## Revendications

1. Bande métallique coulée rapidement trempée., comportant une multiplicité de portions métalliques coulées différentes rapidement trempées, chaque portion étant liée métallurgiquement par alliage lors de la coulée à une portion adjacente le long de longueur de la bande, caractérisée en ce que cette multiplicité de portions (a, b, c, d; a₁, b, a₂) sont des portions différentes d'au moins deux compositions différentes, et en ce que chaque portions est liée métallurgique ment par alliage lors de la coulée à une portion différente latéralement adjacente le long des bords adjacents de ces portions différentes.

2. Bande selon la revendication 1, dans laquelle au moins deux portions adjacentes de cette bande ont une disposition atomique dissemblable.

3. Bande selon la revendication 2, dans laquelle au moins une portion différente de la bande est amorphe (comme défini précédemment).

4. Bande selon la revendication 2 ou la revendication 3, dans laquelle au moins une portion différente de la bande est cristalline.

5. Bande selon l'une quelconque des revendications précédentes, dans laquelle la liaison métallurgique par alliage est formée au niveau d'une zone de transition qui est amorphe (comme défini précédemment) et dans laquelle les portions différentes adjacentes à cette zone de transition sont cristallines.

6. Bande selon l'une quelconque des revendications 1 à 4, dans laquelle des portions différentes adjacentes sont amorphes (comme défini ci-dessus) et la liaison métallurgique par alliage est formé entre elles au niveau d'une zone de transition qui est cristalline.

7. Bande selon l'une quelconque des revendications précédentes, dans laquelle au moins une portion différente de la bande est de l'acier inoxydable.

8. Bande selon l'une quelconque des revendications précédentes, dans laquelle au moins deux portions adjacentes de cette bande ont des épaisseurs différentes.

9. Bande selon l'une quelconque des revendications précédentes, dans laquelle au moins deux portions adjacentes de cette bande ont des caractéristiques de résistance à la corrosion différentes.

10. Bande selon l'une quelconque des revendications précédentes, dans laquelle au moins deux portions adjacentes de cette bande ont des caractéristiques électriques différentes.

11. Bande selon l'une quelconque des revendications précédentes, dans laquelle au moins deux portions adjacentes de cette bande ont des caractéristiques de dilatation différentes.

12. Bande selon l'une quelconque _{'}des revendications précédentes, dans laquelle au moins une portion comporte un alliage ayant des constituants majeurs choisis parmi le fer, le nickel, le cobalt et leurs mélanges, et des constituants mineurs choisis parmi le silicium, le bore, le phosphore, le carbone, l'aluminium, le vanadium, le béryllium, le chrome et leurs mélanges, avec des impuretés accidentelles.

13. Bande selon l'une quelconque des revendications précédentes, dans laquelle au moins une portion est amorphe (comme défini ci-dessus) et a une composition de Fe₈₀₋₈₅, Si₃₋₇, B₁₀₋₁₅, sur la base des pourcentages atomiques.

14. Bande selon l'une quelconque des revendications précédentes, dans laquelle au moins une portion est amorphe (comme défini ci-dessus) et a une composition de Fe₃₆₋₄₃ Ni₃₆₋₄₃ B₁₇₋₂₂, sur la base des pourcentages atomiques.

15. Bande selon l'une quelconque des revendications précédentes, dans laquelle au moins une portion est amorphe (comme défini ci-dessus) et a une composition de Fe₈₀ B₁₂ Si₈, sur la base des pourcentages atomiques.

16. Bande selon l'une quelconque des revendications précédentes, dans laquelle au moins une portion est amorphe (comme défini ci-dessus) et a une composition de Fe₇₉ B₁₅ Si₆, sur la base des pourcentages atomiques.

17. Bande selon l'une quelconque des revendications précédentes, dans laquelle au moins une portion est amorphe (comme défini ci-dessus) et a une composition de Fe₈₁, B₁₃ Si₅ C,, sur la base des pourcentages atomiques.

18. Bande selon l'une quelconque des revendications précédentes, dans laquelle au moins une portion est amorphe (comme défini ci-dessus) et a une composition de Fe₈₄ B₁₅ Si₁, sur la base des pourcentages atomiques.

19. Bande selon l'une quelconque des revendications précédentes, dans laquelle la liaison métallurgique est formée au niveau d'une zone de transition entre des portions ayant une largeur inférieure à 1,5 mm.

20. Bande selon l'une quelconque des revendications précédentes, dans laquelle la liaison métallurgique est formée au niveau d'une zone de transition entre des portions ayant une largeur inférieure à cinq fois l'épaisseur moyenne des portions liées.

21. Bande selon l'une quelconque des revendications précédentes, dans laquelle la liaison métallurgique est formée au niveau d'une zone de transition ayant une résistance mécanique supérieure à celle des deux portions liées adjacentes.

22. Bande selon l'une quelconque des revendications 1 à 20, dans laquelle la liaison métallurgique par alliage est formée au niveau d'une zone de transition ayant une résistance mécanique inférieure à celle des deux portions liées adjacentes.

23. Procédé pour couler une bande métallique ayant une multiplicité de portions différentes métallurgiquement liées par alliage le long de la longueur de cette bande, consistant à amener une multiplicité de courants de métal en fusion à partir d'une multiplicité de tuyères sur une surface de coulée et de trempe rapide se déplaçant à une vitesse comprise entre 61 et 3048 mètres par minute au droit de ces tuyères, caractérisé en ce qu'on dépose un premier courant (20) d'un premier métal en fusion sur cette surface de coulée (18) à partir d'une tuyère (10a) d'un premier creuset (10) et qu'on dépose à côté du premier courant au moins un courant additionnel (22) d'un deuxième métal en fusion différent depuis une tuyère (11a) d'un deuxième creuset (11) sur cette surface de coulée (18) de façon qu'une portion de bord périphérique du courant additionnel (ou des courants additionnels) soit en contact avec une portion de bord périphérique d'un métal différent adjacent pour créer entre eux une . liaison métallurgique par alliage lors de la coulée.

24. Dispositif pour couler des bandes métalliques ayant une multiplicité de portions différentes métallurgiquement liées par alliage le long de la longueur de la bande, comportant des moyens de creusets pour recevoir et maintenir du métal en fusion et ayant une multiplicité de tuyères à travers lesquelles une multiplicité de courants de métal en fusion peut être amenée de ces moyens sur une surface de coulée et de trempe rapide disposée à moins de 3,048 mm des tuyères et se déplaçant au droit des tuyères à une vitesse comprise entre 61 et 3048 mètres par minute, caractérisé en ce que ces moyens de creusets comprennent un premier creuset (10) ayant une cavité intérieure pour recevoir et maintenir un métal en fusion et une tuyère (10a) à travers laquelle un premier courant (20) de métal en fusion peut être amené de sa cavité et déposé sur la surface de coulée (18), et au moins un creuset additionnel (11) ayant une cavité intérieure pour recevoir et maintenir un métal en fusion et une tuyère ( 1 a) à travers laquelle au moins un courant additionnel (22) d'un deuxième métal en fusion différent peut être amené depuis sa cavité et déposé sur la surface de coulée (18), ce creuset additionnel (11) ayant sa tuyère (11a) disposée sur le côté de la première de telle sorte qu'une portions de bord périphérique du courant additionnel (22) vienne en contact avec une portion de bord périphérique d'un métal différent adjacente pour créer entre elles une liaison métallurgique par alliage lors de la coulée.

25. Dispositif selon la revendication 24, dans lequel le ou les creusets (10, 11) sont réalisés en un matériau résistant au métal en fusion choisi parmi les suivants: silice, alumine, graphite, mélange graphite alumine, mélange graphite argile, argile à feu, quartz, nitrure de bore, nitrure de silicium, carbure de silicium, carbure de bore, zircone, silicate de zirconium stabilisé, magnésie, magnésite au chrome, kaolin fibreux et leurs combinaisons.

26. Dispositif selon la revendication 24 ou 25, dans lequel au moins une portion de la tuyère (10a, 11 a) du creuset (10, 11) est construite en un matériau résistant au métal en fusion choisi parmi les suivants: silice, alumine, graphite, mélange graphite alumine, mélange graphite argile, argile à feu, quartz, nitrure de bore, nitrure de silicium, carbure de silicium, carbure de bore, zircone, silicate de zirconium stabilisé, magnésie, magnésite au chrome, kaolin fibreux et leurs combinaisons.

## Patentansprüche

1. Schnell abgeschrecktes, gegossenes metallisches Band, mit einer Vielzahl von ungleichartigen, schnell abgeschreckten, gegossenen, metallischen Bereichen, wobei jeder Bereich metallurgisch während des Gießens mit einem benachbarten Bereich in Längsausdehnung des Bandes legiert-verbunden wird, dadurch gekennzeichnet, daß die Vielzahl von Bereichen (a, b, c, d; a₁, b, a₂) ungleichartige Bereiche aus wenigstens zwei verschiedenen Zusammensetzungen sind, und daß jeder Bereich metallurgisch während des Gießens mit einem seitlich benachbarten ungleichartigen Bereich entlang den benachbarten Rändern der ungleichartigen Bereiche legiert-verbunden ist.

2. Band nach Anspruch 1, bei dem wenigstens zwei benachbarte Bereiche des Bandes eine ungleichartige Atomanordnung aufweisen.

3. Band nach Anspruch 2, bei dem wenigstens ein ungleichartiger Bereich des Bandes amorph ist (wie zuvor definiert).

4. Band nach Ansprüchen 2 oder 3, bei dem wenigstens ein ungleichartiger Bereich des Bands kristallin ist.

5. Band nach einem der vorhergehenden Ansprüche, bei dem die metallurgische Legierungsgrenze in einer Übergangszone ausgebildet ist, die amorph ist (wie zuvor definiert) und bei dem die ungleichartigen Bereich neben dieser Übergangszone kristallin sind.

6. Band nach einem der Ansprüche 1 bis 4, bei dem benachbarte ungleichartige Bereiche amorph sind (wie zuvor definiert) und die metallurgische Legierungsgrenze in einer dazwischenliegenden Übergangszone ausgebildet ist, welche kristallin ist.

7. Band nach einem der vorhergehenden Ansprüche, bei dem wenigstens einer der ungleichartigen Bereiche des Bandes aus rostfreiem Stahl besteht.

8. Band nach einem der vorhergehenden Ansprüche, bei dem wenigstens zwei benachbarte Bereiche des Bandes unterschiedliche Dicken aufweisen.

9. Band nach einem der vorhergehenden Ansprüche, bei dem wenigstens zwei benachbarte Bereiche des Bandes ungleichartige Korrosionswiderstandseigenschaften aufweisen.

10. Band nach einem der vorhergehenden Ansprüche, bei dem wenigstens zwei benachbarte Bereiche des Bandes ungleichartige elektrische Eigenschaften aufweisen.

11. Band nach einem der vorhergehenden Ansprüche, bei dem wenigstens zwei benachbarte Bereiche des Bandes ungleichartige Ausdehnungseigenschaften aufweisen.

12. Band nach einem der vorhergehenden Ansprüche, bei dem wenigstens ein Abschnitt eine Legierung enthält, deren Hauptbestandteile ausgewählt sind aus Eisen, Nickel, Kobalt und deren Mischungen und deren Nebenbestandteile aufgewählt sind aus Silizium, Bor, Phosphor, Kohlenstoff, Aluminium, Vanadium, Beryllium, Chrom und deren Mischungen, mit geringfügigen Verunreinigungen.

13. Band nach einem der vorhergehenden Ansprüche, bei dem wenigstens ein Bereich amorph ist (wie zuvor definiert) und die Zusammensetzung, in Gewichtsprozenten, Fe₈₀₋₈₅-Si₃₋₇B₁₀₋₁₅ aufweist.

14. Band nach einem der vorhergehenden Ansprüche, bei dem wenigstens ein Bereich amorph ist (wie zuvor definiert) und die Zusammensetzung, in Gewichtsprozenten, Fe₃₆-₄₃-Ni₃₆₋₄₃B₁₇₋₂₂ aufweist.

15. Band nach einem der vorhergehenden Ansprüche, bei dem wenigstens ein Bereich amorph ist (wie zuvor definiert) und die Zusammensetzung, in Gewichtsprozenten, Feₛₒ-B₁₂Siₛ aufweist.

16. Band nach einem der vorhergehenden Ansprüche, bei dem wenigstens ein Bereich amorph ist (wie zuvor definiert) und die Zusammensetzung, in Gewichtsprozenten, Fe₇₉-B₁₅Si₈ aufweist.

17. Band nach einem der vorhergehenden Ansprüche, bei dem wenigstens ein Bereich amorph ist (wie zuvor definiert) und die Zusammensetzung, in Gewichtsprozenten, Feₛ,-B₁₃Si₅C₁ aufweist.

18. Band nach einem der vorhergehenden Ansprüche, bei dem wenigstens ein Bereich amorph ist (wie zuvor definiert) und die Zusammensetzung, in Gewichtsprozenten, Fes4-B₁₅Si₁ aufweist.

19. Band nach einem der vorhergehenden Ansprüche, bei dem die metallurgische Grenze in einer Übergangszone ausgebildet ist zwischen Bereichen, deren Breite weniger als fünfmal 1,5 mm beträgt.

20. Band nach einem der vorhergehenden Ansprüche, bei dem die metallurgische Grenze in einer Übergangszone ausgebildet is zwischen Bereichen, deren Breite weniger also fünfmal durchschnittliche Dicke der miteinander verbundenen Abschnitte ist.

21. Band nach einem der vorhergehenden Ansprüche, bei dem die metallurgische Grenze in einer Übergangszone ausgebildet ist, deren mechanische Festigkeit größer als diejenige der beiden benachbarten verbunden Bereiche ist.

22. Band nach einem der vorhergehenden Ansprüche 1 bis 20, bei dem die metallurgische Legierungsgrenze in einer Übergangszone ausgebildet ist, deren mechanische Festigkeit geringer als diejenige der beiden benachbarten verbundenen Bereiche ist.

23. Verfahren zum Gießen eines metallischen Bandes, das eine Vielzahl von ungleichartigen Bereichen aufweist, die metallurgisch entlang den Längsausdehnungen des Bandes miteinander legiertverbunden sind, wobei eine Vielzahl von geschmolzenen Metallströmen aus einer Vielzahl von Düsen auf eine sich schnell abkühlende Gießfläche gerichtet werden, das sich mit einer Geschwindigkeit zwischen 61 und 3048 Meter pro Minute (200 bis 10,000 Fuß/ min Umfangsgeschwindigkeit) an den Düsen vorbeibewegt, gekennzeichnet, durch das Aufbringen eines ersten Strahls (20) eines ersten geschmolzenen Metalls auf die Gießoberfläche (18) aus einer Düse (10a) eines ersten Gießtiegels (10) und Aufbringen seitlich neben dem ersten wenigstens eines zusätzlichen Stromes (22) eines zweiten, verschiedenen geschmolzenen Metalls aus einer Düse (11 a) eines zweiten Gießtiegels (11) auf die Gießoberfläche (18), derart, daß ein Längsrandabschnitt des genannten wenigstens einen zusätzlichen Stroms einen Längsrandabschnitt eines benachbarten unterschiedlichen Metalls berüht, um so eine metallurgische Legierungs-Bindung zwischen ihnen während des Gießens auszubilden.

24. Vorrichtung zum Gießen eines metallischen Bandes, das eine Vielzahl von ungleichartigen Bereichen aufweist, die metallurgisch miteinander entlang der Längsausdehnung des Bandes legiert-verbunden sind, welche Gießanordnungen aufweist zur Aufnahme und Aufbewahren geschmolzenen Metalls und eine Vielzahl von Düsen besitzt, durch welche eine Vielzahl von Strömen von geschmolzenem Metall aus der genannten Anordnung auf eine sich schnell abkühlende Gießoberfläche gegeben werden kann, welche im Bereich innerhalb 3,048 mm (0,120 Zoll) vor den Düsen angeordnet ist und sich an den Düsen entlang mit einer Geschwindigkeit von 61 bis 3048 Metern pro Minute (200 bis 10.000 Fuß/min Umfangsgeschwindigkeit) bewegen kann, dadurch gekennzeichnet, daß die Gießanordnung einen ersten Gießtiegel (10) aufweist, mit einem Innenraum zur Aufnahme und zum Aufbewahren von geschmolzenem Metall und eine Düse (10a) aufweist, durch welche ein erster Strom (20) aus geschmolzenem Metall aus dem Innenraum abgegeben werden kann und auf eine Geißoberfläche (18) aufgebracht werden kann und wenigstens einen zusätzlichen Gießtiegel (11) aufweist mit einem Innenraum zur Aufnahme und zum Aufbewahren von geschmolzenem Metall und mit einer Düse (1 1a), durch welche wenigstens ein zusätzlicher Strom (22) eines zweiten verschiedenen geschmolzenen Metalls aus dem Innenraum abgegeben werden kann und auf eine Gießoberfläche (18) aufgebracht werden kann, wobei die Düse (11 a) des wenigstens einen zusätzlichen Gießtiegel (11) seitlich der ersten derart angeordnet ist, dß ein Längsrandabschnitt des wenigstens einen zusätzlichen Stroms (22) einen Längsrandabschnitt des benachbarten unterschiedlichen Metalls berührt um eine metallurgische Legierungsgrenze zwischen ihnen während des Gießens zu bilden.

25. Vorrichtung nach Anspruch 24, bei der wenigstens einer der Gießtiegel (10, 11) aus einem das flüssige Metall aushaltenden Material gebildet ist, das ausgewählt ist aus Silika, Aluminiumoxid, Graphit, Aluminiumoxid-Graphit, Ton-Graphit, Feuerton, Quarz, Bomitrid, Siliziumnitrid, Siliziumcarbid, Borcarbid, Zirkondioxid, stabilisiertes Zirkonsilikat, Magnesiumcarbonat, Chrom-Magnesit, faserförmiges Kaolin und deren Mischungen.

26. Vorrichtung nach Anspruch 24 oder 25, bei der wenigstens ein Teil der Düse (1 Oa, 11 a) wenigstens eines Gießtiegels (10, 11) aus einem flüssiges Metall aushaltenden Material besteht, das ausgewählt ist aus Silika, Aluminiumoxid, Graphit, Aluminiumoxid-Graphit, Ton-Graphit, Feuerton, Quarz, Bornitrid, Siliziumnitrid, Siliziumcarbid, Borcarbid, Zirkondioxid, stabilisiertes Zirkonsilikat, Magnesiumcarbonat, Chrom-Magnesit, faserförmiges Kaolin und deren Mischungen.
